

No. 651,705.

Patented June 12, 1900.

M. H. FLETCHER.

CORE AND METHOD OF MAKING SAME.

(Application filed Jan. 18, 1898.)

(No Model.)



# UNITED STATES PATENT OFFICE.

MORDECAI H. FLETCHER, OF CINCINNATI, OHIO.

## CORE AND METHOD OF MAKING SAME.

SPECIFICATION forming part of Letters Patent No. 651,705, dated June 12, 1900.

Application filed January 13, 1896. Serial No. 575,265. (No model.)

*To all whom it may concern:*

Be it known that I, MORDECAI H. FLETCHER, a citizen of the United States, residing at Cincinnati, Ohio, have invented new and useful Improvements in Cores and the Method of Making the Same, of which the following is a specification.

My invention relates to methods of manufacturing cores employed in casting hollow articles—such, for example, as hollow cylinders—wherein a core-surface of sand and loam is superimposed upon a core-bar of metal. In forming such cores for casting pipe, &c., for water and gas mains and similar cylindrical objects the ordinary practice is to first enwrap the core-bar with a rope of hay in adjacent convolutions and upon this place a coating of plastic clay, upon which, when dried, is placed a final concentric layer of "loam," forming the surface of the core for casting. There is thus produced a combustible foundation layer for the clay and loam, which is burned away by the heat of the molten metal, thus leaving space between the clay layer and the core-bar, facilitating the escape of the gases engendered in casting and enabling the core-bar to be withdrawn. The earthy layers being thus left without support may be broken from the interior of the casting. Besides the expense of manipulation and the cost of material destroyed, this method of procedure is subject to further objection in this, namely, that the layer formed by the hay rope is unequally compressible and produces irregularity in the contour and dimensions of the casting under the compression of the molten metal, often seriously impairing the resulting product. Again, the interstices of the hay-rope windings are not uniform and often allow the clay layer to seat against the core-bar, and thus the hardening of the earthy layers and the shrinkage of the casting render the withdrawal of the core-bar difficult or impossible without breakage or serious injury to the casting.

The object of my invention is to provide a novel method of manufacturing a core which avoids the expense of hay rope, also the clay layer applied to the rope, and that shall be free from the objectionable features named and more rigid and efficient, thereby not only economizing in cost, but producing castings

of superior uniformity of dimensions and quality and avoiding the loss due to imperfect cores.

To this end my invention consists in the method of making a core built upon a core-bar in which the hay rope is replaced by a foundation layer of earthy matter having a sufficient proportion of combustible material disseminated through the same to render it extremely porous and friable when subjected to the heat of the casting, so that the core may be readily withdrawn. The core so made requires but a thin outer surfacing-coat of loam, which is therefore easily broken from the casting.

In the drawings attached hereto, illustrating the structural features of a core applied to the casting of water or gas pipe, Figure 1 exhibits a partial axial section of a flask prepared for the reception of molten metal with the core in place, Fig. 2, a horizontal cross-section of the same parts in the plane  $\alpha$  of Fig. 1.

In the drawings, F designates a flask prepared for the casting of a pipe in the space s, and A the core-bar suited to the inner contour of the pipe to be cast.

For the purpose of my invention the core-bar A is a cylindrical casting of metal, usually hollow, having a large number of vent-openings  $\sigma$  through the shell. Immediately upon the perforated surface of the core-bar I place a layer B of material formed and applied as follows: The material of this layer is preferably about one-third part pulverized earthy material (such as the spent core-dirt of the pipe works) and two-thirds comminuted woody combustible material, thoroughly mixed and worked into a plastic mass, somewhat adhesive, with water and applied as a concentric layer directly upon the surface of the core-bar. The earthy material may contain a sufficiency of loam or of mineral cement to render the ultimate mass somewhat adhesive to and reasonably firm, when dried, upon the core-bar. The combustible material may be sawdust, ground leaves, straw, seaweed, &c., or any cheap material of this nature capable of being disseminated in a finely-divided state throughout the mass, or spent core-dirt may be used in connection with mucilaginous matter otherwise introduced—as, for example, a

55

60

70

75

80

85

90

95

100

mixture of horse-manure with the sawdust or other combustible matter—but in general loam will be preferred. The application to the core is made substantially in the same 5 manner and by the means of the usual appliances (not shown) now employed for applying the outer layer of clay over the hay rope, or may be applied by means of a flexible web, such as is sometimes employed in the manu- 10 facture of earthen pipe, and when applied the layer is dressed to a uniform thickness and comparatively smooth surface. It is then thoroughly dried to expel moisture. Inasmuch as the layer contains so large a pro- 15 portion of woody fiber, which is very absorbent, the mass as made contains an excess of moisture, the drying out of which renders it firm and exceedingly porous. After the preparation of the inner layer as described a thin 20 finishing-coat *b* of loam is applied in the usual manner and dressed to a true cylindrical surface throughout. The core is then subjected to a second drying and is finished in the usual manner. There is thus produced a core con- 25 sisting of the core-bar A, a layer of partially-combustible material B surrounding the same, and the outer layer *b* of loam forming the finished and smooth exterior. The large proportion and uniform distribution of the woody 30 constituents of the initial layer renders it exceedingly porous in its dry state, and this constituent being combustible is consumed by the intense heat of the adjacent molten metal of the casting, thus rendering the inner layer 35 extremely friable.

The disintegration of the layer B during the casting operation is sufficiently slow to enable the outer layer *b* to retain its proper form until the metal "sets," while at the same time

the inner layer is sufficiently porous, in connection with the apertures *o*, to afford the proper vent for the gases engendered in casting and also to freely admit air to effect combustion of the combustible material of the inner layer B. 45

As a result of the proper application of the invention the construction of cores is considerably economized and more accurate and uniform castings are produced, besides largely decreasing the percentage of failures or imperfect castings. 50

The composition, both as to character and proportion of the constituents, of the initial layer B may also vary largely, according to local conditions and conveniences. The general aim is to employ the most inexpensive materials, and those designated have been found to work well in practice. 55

I claim as my invention and desire to secure by Letters Patent of the United States— 60

The improvement in the art of forming cores for casting hollow cylinders, pipe, &c., consisting in first coating the perforated core-bar with a plastic adhesive mass of moist earthy material containing a large percentage 65 of combustible material in comminuted state; then drying the same to set and render it porous; and lastly covering the said coating with a finishing-coat of loam, and drying the same in the usual manner, substantially as set 70 forth.

In testimony whereof I have hereunto set my hand in the presence of two subscribing witnesses.

MORDECAI H. FLETCHER.  
Witnesses:

L. M. HOSEA,  
FRANK K. BOWMAN.